

Nov. 16, 1926.

1,607,089

F. H. LEIDECKER

METHOD OF MANUFACTURING SPIRAL DRILLING BITS AND THE LIKE

Filed Oct. 27, 1925

*Fig. 1.*



*Fig. 4.*



*Fig. 2.*



*Fig. 5.*



*Fig. 6.*



*Fig. 3.*



F. H. Leidecker  
Inventor

By *Cadmore & Co.*  
Attorneys

Patented Nov. 16, 1926.

1,607,089

# UNITED STATES PATENT OFFICE.

FOSTER H. LEIDECKER, OF MARIETTA, OHIO, ASSIGNOR TO THE LEIDECKER TOOL CO., OF MARIETTA, OHIO.

## METHOD OF MANUFACTURING SPIRAL DRILLING BITS AND THE LIKE.

Application filed October 27, 1925. Serial No. 65,198.

This invention relates to a method of making spiral drilling bits and like devices such as used, for example, in well drilling operations.

5 The invention relates more especially to a method of producing bits which, in cross sectional contour, have substantially the appearance of a Maltese cross, the several steps of the method being designed to produce a bit or the like each rib or wing of which will be kept in proper shape during the twisting operation and not become distorted when elongated by a twisting operation.

15 With the foregoing and other objects in view the invention consists in certain novel steps in the method of producing spiral drilling bits and the like, which will be herein-after more fully described and pointed out in the claims, it being understood that various changes may be made without departing 20 from the spirit of the invention as claimed.

In the accompanying drawings I have shown some dies used in carrying out the method and have also shown the article produced.

25 In said drawings,

Figure 1 is a perspective view of a forging die by means of which the billet is given its initial shape prior to the twisting operation.

30 Figure 2 is a perspective view of the twisting die, the position of the billet therein being indicated by broken lines.

Figure 3 is a perspective view of one of the members of the twisting die.

35 Figure 4 is a transverse section through the billet as it appears after the forging operation.

Figure 5 is a similar view showing the spiral drilling bits or the like produced by 40 the action of the twisting die.

Figure 6 is an elevation of a portion of the billet after being acted on by the forging dies.

45 Figure 7 is a similar view showing the partially formed spiral ribs or wings produced by the twisting dies.

Figure 8 is a view of a portion of completed spiral drilling bit.

For the purpose of carrying out the method 50 constituting the present invention there are provided two sets of dies. One set of these dies is used for forging the stock to shape prior to the twisting operation while the dies of the other pair are employed for imparting a twist to the wings or ribs of the

tool. These two sets of dies can be actuated simultaneously in a single machine or in separate machines or, if preferred, can be separately operated. The forging dies have been illustrated in Figure 1 and consist of 60 the cooperating members 1 and 2 the meeting faces of which are recessed as at 3 to provide oppositely extending lateral spaces 4 separated by superposed oppositely extending recess 5 extending into the dies. The end 65 walls of the recesses 5 are preferably concaved transversely as shown at 6 while the side walls of these recesses diverge toward the spaces 4 and merge, along rounded shoulders 7, into the walls of said spaces. The 70 diverging walls of the recesses 5 have been indicated at 8 while those walls of the spaces 4 extending from the rounded shoulders 7 have been indicated at 9. These walls 9 diverge from the recesses 5 and terminate at 75 the end walls 10 which converge to the meeting faces of the dies 1 and 2 where they come together. In practice the distance from *a* to *b* in Figure 1 is equal to the distance between *c* and *d* in said figure. The reason for 80 this will be hereinafter explained.

The twisting dies have been indicated at 10 and 11 in Figure 2 and are provided with recesses 12 in their meeting faces for the reception of the shaped billet received from 85 the dies 1 and 2. In each of the recesses 12 is formed a tapered obliquely disposed fuller 13 designed to enter between the wings or ribs of the formed billet and impart a spiral twist thereto.

The billet to be formed into a spiral drilling bit or the like is placed between and shaped by the dies 1 and 2 and will be given the cross sectional contour outlined by the walls of the several recesses within said dies. 95 Thereafter the billet is given a one-quarter turn and again subjected to the action of the dies. By this last operation those wings or ribs of the billet previously formed within the spaces 4 will have their longitudinal edge portions rounded by the concave end walls 6 of the recesses 5 while the sides of the wings or ribs previously shaped in the recesses 5 will be pressed together. The foregoing operations are repeated, the billet 105 being fed forwardly step by step. Consequently the billet will assume the cross sectional contour illustrated in Figure 4 wherein the wings or ribs are formed with rounded outer faces 14 and inwardly converging 110

side walls 15. The core 16 of the billet thus formed will be over-size. By now placing the billet between and subjecting them to the action of the dies 10 and 11, the opposed fullers 13 will impart twists to two of the wings and, during this twisting operation, will displace some of the metal of the core 16 so that it will flow into the wings being twisted and compensate for the stretch which 10 results from the elongation thereof due to twisting. Thus the wings will not become distorted but will maintain their cross sectional contour. After two of the wings have thus been given a twist for a portion of their 15 length the billet is rotated through one-fourth of a circle and again subjected to the action of the dies 10 and 11. The remaining two wings will thus be twisted and metal displaced from the core into them to 20 serve the cross sectional contours of the wings. Thereafter the billet is fed forwardly step by step between the dies and the foregoing operation repeated until the wings have been twisted throughout their lengths. 25 The displacement of metal from the core into the wings will of course reduce the size of the core so that the cross sectional contour of the tool will be changed from that illustrated in Figure 4 to approximately the contour shown in Figure 5. In this figure as well as 30 in Figures 6, 7 and 8, the wings have been illustrated at 17. Figure 6 shows a portion of the billet after it has been forged to the shape shown in Figure 4 while Figure 7, as 35 heretofore explained, shows the billet partly twisted after it has been acted on one or more times by the dies 10 and 11. A portion of the completed tool has been illustrated in Figure 8. The particular configuration of the spiral drilling bit has certain 40 advantages over other forms of tools of this type but as this particular drilling bit or the like constitutes no part of the present invention it is not deemed necessary to point out the advantages at this time. The greatest 45 objection to producing a drilling bit having the cross sectional contour herein disclosed has been in the difficulty in produc-

ing the tools by a forging method. By providing dies such as described and using them 50 in the manner set forth tools of this character having wings of special cross sectional contours can be produced readily by forging and, because of the displacement of metal into the wings during the twisting 55 operation, said wings or ribs will maintain their contours even though elongated when twisted.

What is claimed is:

1. The herein described method of producing spiral drilling bits and the like which consists in forging a billet to produce wings of predetermined cross sectional contour and an over-size core, and thereafter simultaneously twisting the wings and forcing thereinto surplus metal from the core to compensate for elongation of the wings due to twisting. 60

2. The herein described method of producing spiral drilling bits and the like which includes forging a billet to produce wings having substantially the cross sectional contour of the wings of the finished tool, the core of the billet being over-size, and thereafter subjecting the billet to the action of twisting dies for imparting a twist to the wings and reducing the size of the core, the surplus metal of the core being directed into the wings to compensate for elongation of the wings due to twisting, thereby to maintain the predetermined cross sectional contour of the wings. 70

3. The herein described method of producing spiral drilling bits and the like which consists in producing a billet having an over-size core and radial wings, and thereafter feeding the billet intermittently between twisting dies, said dies operating to simultaneously twist the wings of the billet and displace surplus metal from the over-size core into the wings, thereby to compensate for the elongation of the wings due to twisting. 85

In testimony that I claim the foregoing as my own, I have hereto affixed my signature.

FOSTER H. LEIDECKER.